

# UNITED STATES PATENT OFFICE.

EDWARD D. FROHMAN, OF PITTSBURGH, PENNSYLVANIA.

## REFRACTORY MATERIAL.

1,327,758.

No Drawing.

Application filed April 26, 1919. Serial No. 292,827.

Specification of Letters Patent. Patented Jan. 13, 1920.

*To all whom it may concern:*

Be it known that I, EDWARD D. FROHMAN, residing at Pittsburgh, in the county of Allegheny and State of Pennsylvania, a citizen of the United States, have invented or discovered certain new and useful Improvements in Refractory Materials, of which improvements the following is a specification.

10 As is well known in the art, a mixture of fire clay and silicious material, such as ganister, asbestos, etc., will begin to coalesce at about 2500 degrees F. and that by adding silicate of soda to such a mixture a permanent binding of the materials will begin at a lower temperature, dependent upon the amount of silicate of soda added. The objection to this mixture is the difficulty of preparing it for use at the point of use on 20 account of the slow solubility of the silicate of soda.

The object of the invention described herein is to provide a mixture of fine clay, silicious material and another material 25 which is readily soluble in water and when so dissolved will form a binder having an efficiency equal to that of the silicate of soda.

Shipment of materials mixed with silicate of soda requires the employment of liquid 30 tight receptacles and freight must be paid on the liquid contents, whereas the mixture claimed herein may be shipped in any kind of receptacles which will protect it from moisture and no freight is paid on mere liquid.

In the practice of the invention fire clay and a silicious material as ganister or asbestos in a powdered or finely divided condition and finely divided wood pulp refuse or

sulfite pitch are thoroughly mixed together. 40 The fire clay and silicious material may be used in equal or any desired relative proportions and dry wood pulp refuse or sulfite pitch is added in amounts varying from one to ten per cent. of the entire mass of other 45 materials. The percentage of binder depends upon the coarseness of the ganister, the coarser the grains the greater the percentage of binder required.

This mixture of materials can be readily 50 shipped to the point of use and rendered capable of use merely by the addition of water in quantities dependent upon the consistency desired.

As is well known in the art, a mixture of 55 fire clay and silicious material can be rendered plastic by the addition of water, but when such a mass is dried out it cracks and crumbles. When silicate of soda is used as a binder no cracking or crumbling will occur 60 and the same is true of the mixture claimed herein, which however has the advantage that it may and can be shipped in a dry condition and prepared for use by the addition of water. 65

I claim herein as my invention:

1. A refractory material consisting of a mixture of finely divided dry fire clay, silicious material and sulfite pitch.

2. A refractory material consisting of a 70 mixture of finely divided fire clay, silicious material, sulfite pitch and water.

3. A refractory material consisting of a mixture of finely divided dry fire clay, ganister and sulfite pitch. 75

In testimony whereof I have hereunto set my hand.

EDWARD D. FROHMAN.